

3,702,829

MICROSCOPIC CAPSULES AND PROCESS OF  
MAKING SAMELloyd D. Taylor, Everett, Mass., assignor to Polaroid  
Corporation, Cambridge, Mass.No Drawing. Original application Mar. 25, 1963, Ser. No.  
267,847, now Patent No. 3,396,026, dated Aug. 6,  
1968. Divided and this application May 15, 1968, Ser.  
No. 729,397

Int. Cl. B01j 13/02; B44d 1/02

U.S. Cl. 252—316

4 Claims

## ABSTRACT OF THE DISCLOSURE

Microscopic capsules having walls which include a substantially continuous polymeric layer comprising a coacervate containing a low isoelectric point gelatin and a gelatin derivative, which derivative comprises the reaction product of gelatin and a carboxylated derivatizing agent which will not substantially cross-link said gelatin, and which reacts with at least a portion of the gelatin's amino groups, surrounding a nucleus comprising a water-immiscible medium.

The instant application is a division of copending U.S. application of Lloyd D. Taylor, Ser. No. 267,847, filed Mar. 25, 1963, now U.S. Pat. No. 3,396,026.

The application of William J. McCune, Jr., filed May 9, 1961, Ser. No. 108,774, now U.S. Pat. No. 3,276,869, discloses the use of minute capsules for use in photographic processes. In one embodiment, the minute capsules contain dye developers for use in preparing color images by the diffusion transfer process. In another embodiment, the microscopic capsules are coated with a layer of silver halide. U.S. Pat. No. 2,983,606, issued May 9, 1961, to Howard G. Rogers, discloses processes employing dye developers to form color transfer images and products useful therein. The application of Edwin H. Land and Howard G. Rogers, Ser. No. 565,135, filed Feb. 13, 1956, now U.S. Pat. No. 3,345,163 discloses the use of such dye developers in integral multilayer negatives to give multicolor transfer images.

Accordingly, it is one object of this invention to provide novel minute capsules for use in the photographic products and processes.

Another object of this invention is to provide minute capsules whose walls comprise photographic gelatin.

Still another object of this invention is to provide novel processes for the preparation of minute capsules.

Still another object of this invention is to provide capsules of the aforementioned structure wherein color-providing materials are encapsulated.

Other objects of the invention will in part be obvious and will in part appear hereinafter.

The invention accordingly comprises the process involving the several steps and the relation and order of one or more of such steps with respect to each of the others, and the product possessing the features, properties and the relation of elements which are exemplified in the following detailed disclosure, and the scope of the application of which will be indicated in the claims.

For a fuller understanding of the nature and objects of the invention, reference should be had to the following detailed description.

Methods of preparation of microscopic, pressure-rupturable capsules containing a water-immiscible medium are well known to the art. Generally such capsules are formed by deposition of a complex colloid material around microscopic droplets of a water-immiscible medium by the process of causing coacervation, by dilution or

adjustment of the pH, to occur in a mixture of two different colloid salts in which the water-immiscible material is dispersed as droplets, and then gelling the complex colloid. Generally, a complex colloid material is formed

5 of an aqueous solution of one colloid, emulsifying the nuclei material or internal phase therein and mixing the thus-formed emulsion with an aqueous salt of another colloid. Alternatively the two colloid materials may be made and mixed and the water-immiscible material emulsified therein. Coacervation is then brought about by dilution and/or by adjusting the pH of the mixture. The gellable colloid materials used in the solutions must be ionizable and the art has taught that the sols must exist in the mixture with opposite electric charges. One well-known system comprises high isoelectric point gelatin as the positive colloid, gum arabic as the negative colloid, and water. A solution of these materials is prepared and the pH and concentration of the system is adjusted to a point where coacervation occurs. A water-immiscible material may then be added to the solution and the gelatin-gum arabic coacervate phase will deposit around the water-immiscible droplets thereby encapsulating the water-immiscible medium.

In photographic products and processes, low isoelectric point gelatin is preferred as a colloid binder over high isoelectric point gelatin. Accordingly, it becomes considerably more desirable to prepare minute capsules which are to be used in photographic products and processes with low isoelectric point gelatin. Also, gum arabic is not available domestically and problems of supply may arise. Therefore, the problem that presents itself is to replace a positive colloid with a negative colloid and still provide a system in which a coacervate can be formed that is, to provide a multi-component encapsulation system wherein the constituents which provide the encapsulation functionality each possess a net negative charge.

The novel process of this invention comprises encapsulation of water-immiscible materials in low isoelectric point gelatin, particularly photographic grade gelatin, to form minute capsules.

40 In one embodiment of the present invention, the encapsulating wall material comprises low isoelectric point gelatin and, as a second colloid material, a gelatin derivative comprising the reaction product of a dicarboxylic acid anhydride and gelatin.

45 In carrying out the novel process of this invention, a solution of low isoelectric point gelatin is prepared and a solution of a second colloid is added. With constant stirring throughout, the temperature and pH of the system is adjusted to provide a coacervate phase of the gelatin and the second colloid. The water-immiscible internal phase material is then added to the coacervate and the solution is cooled slowly. Capsules are formed by the deposition of the complex colloid comprising gelatin and the second colloid around the droplets of the internal phase. The capsular walls are also hardened by the lowering of the temperature. The thus-formed capsules may then be hardened by appropriate means, for example, rapid cooling and/or the addition of the hardening agent such as glutaraldehyde. The hardened capsules may then be isolated and dried and utilized in the desired appropriate manner.

50 As examples of suitable dicarboxylic acid anhydrides which may be reacted with gelatin to form gelatin derivative reaction products, mention may be made of phthalic anhydride, tri-mellitic anhydride, succinic anhydride and glutaric anhydride. The type of gelatin which is reacted with the dicarboxylic acid anhydride is not critical; high or low isoelectric point gelatin may be used. It should be noted, however, that certain anhydrides are known which will crosslink gelatin. Therefore, these materials

should be avoided when selecting anhydrides to prepare a gelatin product for use as the second colloid in this invention. Gelatin-anhydride reaction products are prepared according to the procedure set forth in U.S. Pat. No. 2,525,753.

It should be understood that the dicarboxylic acid anhydrides suitable for use in this invention may have other carboxylic acid groups as well as the two that make up the anhydride groups.

It should be additionally understood that while gelatin derivatized with dicarboxylic acid anhydrides is one of the preferred materials for use as the second colloid gelatin derivatized with other materials which will react with the amino groups of the gelatin is also useful provided that carboxylic acid groups are also added to the gelatin. For example, gelatin derivatized with p-carboxybenzenesulfonyl chloride may also be suitable for use in this invention as the second colloid.

It has also been found that minute capsules containing photosensitive silver halide salts in the capsule walls can be prepared by the novel process of this invention. The aforementioned capsules comprise gelatin with silver halide deposited therein encapsulating an internal phase material. Gelatin-silver halide capsules may be prepared by forming a coacervate of a solution of gelatin-silver halide emulsion and a second colloid, such as the reaction product of gelatin and a dicarboxylic acid anhydride in accordance with the above-disclosed procedure.

The gelatin-silver halide emulsion is prepared by procedures well known to the art, for example, by reacting a water-soluble silver salt, preferably silver nitrate, with at least one water-soluble halide salt, preferably sodium or potassium bromide, most preferably in combination with sodium or potassium iodide, in an aqueous solution of a low isoelectric point gelatin colloid peptizing agent. Additional preparation and sensitization may be carried out by any of the accepted procedures known to the art.

The terms "sensitive," "photosensitive" and "sensitized" and other terms of similar import are herein employed in the generic sense to describe materials possessing physical and chemical properties which enable them to form usable images when exposed to actinic radiation.

By means of the above-described novel process of this invention, solids as well as solutions and suspensions may comprise the internal phase. Solid materials may then be encapsulated by their methods: (1) by direct encapsulation of a solid, (2) by the encapsulation of a solution of the solid in a volatile solvent, and evaporating the solvent after the formation of the capsule, thereby leaving the solid inside, and (3) by the encapsulation of the solid suspended in a material, preferably an organic solvent which is also immiscible in the aqueous coacervate system.

The following nonlimiting example illustrates the preparation of capsules within the scope of this invention.

#### EXAMPLE

The pH of 173 ml. of 8% aqueous solution of the reaction product of gelatin and phthalic anhydride (prepared according to the method disclosed in U.S. Pat. No. 2,525,753) was adjusted to a pH of 6.5 and added to 700 ml. of water at 45° C. 200 ml. of 10% aqueous solution of low isoelectric point gelatin was adjusted to a pH of 6.5 and added to the gelatin derivative solution. The pH of the combined solution was then adjusted to 4.5 with acetic acid. 190 ml. of toluene was then added to the solution with vigorous agitation and the mixture was then allowed to cool gradually to about 25° C. The temperature of the solution was then dropped rapidly to 10° C with a Dry Ice acetone bath. 10 ml. of glutaraldehyde was then added to the solution and the capsules were isolated and dried.

The copending application of Lloyd D. Taylor, Ser. No. 267,838, filed Mar. 25, 1963, now U.S. Pat. No. 3,369,900, discloses and claims minute capsules whose

walls comprise a single colloid material. It should be understood that a photosensitive silver halide emulsion can be prepared utilizing said single colloid and the thus-prepared colloid can be used in the preparation of capsules which contain silver halide in the capsular walls according to the procedure of the above-noted copending application Ser. No. 267,838, now U.S. Pat. No. 3,369,900.

In preparing capsules by the novel process of this invention, the agitation or stirring action given the colloid system is determinative of the size of the droplets of water-immiscible phase and ultimately the size of the capsules. The more vigorous the stirring action, the smaller the size of the droplet. For example, capsules about 1 to 10 microns in size may be prepared using the stirring action of a Waring Blender. Larger size capsules would be prepared by less vigorous stirring action. Capsules prepared by the novel process of this invention are in the 1 to 100 micron range.

The complex colloid system in this invention utilizes what is essentially two negative colloids at an acid pH. The difference in charge between the colloids is one of degree, not kind.

The novel capsules prepared by the process of this invention which contain color-providing substances or which comprise walls of gelatin containing photosensitive silver halide, the latter of which is disclosed in copending application of Lloyd D. Taylor, Ser. No. 267,847, filed Mar. 25, 1963, now U.S. Pat. No. 3,396,026, are useful in photographic products and processes. For example, such capsules may be used in photosensitive elements disclosed in the above-mentioned copending application, Ser. No. 108,774, now U.S. Pat. No. 3,276,869. It should be understood that, in photographic applications, the internal phase may be extracted from the capsules by an aqueous alkaline solution. Capsules within the scope of the present invention may also be used in printing or reproduction processes. For example, a dye or printing oil may be incorporated into the internal phase prior to coacervation and a layer of the capsules printed on a sheet of paper. By the application of pressure in a particular pattern, the capsules will rupture liberating the dye or oil thus reproducing the original pressure pattern on the paper.

Since certain changes may be made in the above products and processes without departing from the scope of the invention herein involved, it is intended that all matter contained in the above description shall be interpreted as illustrative and not in a limiting sense.

What is claimed is:

1. A process of making microscopic capsules which comprises, in combination, the steps of:
  - (1) providing a fluid mixture which comprises an aqueous solution of a low isoelectric point gelatin comprising a net negative charge and a gelatin derivative, said gelatin derivative comprising the reaction product of gelatin and a carboxylated gelatin derivatizing agent which will not substantially cross-link said gelatin, and which reacts with at least a portion of the amino groups of gelatin to provide neutralization of at least a portion of the positive charges provided to the gelatin molecule, in aqueous solution, by said amino groups, resulting in a derivatized gelatin material comprising a net negative charge, and a water-immiscible medium, whereby droplets of said water-immiscible medium are provided dispersed in said aqueous solution;
  - (2) adjusting the pH and temperature of the fluid mixture to cause coacervation of said gelatin and said derivatized gelatin whereby said coacervate deposits around the individual droplets of said water-immiscible medium, individually encapsulating said droplets; and
  - (3) gelling said coacervate by cooling said capsules below the gelling temperature of said coacervate.
2. The process as defined in claim 1 wherein said

gelatin derivatizing agent comprises a dicarboxylic acid anhydride.

3. Microscopic capsules consisting essentially of a substantially continuous polymeric layer surrounding a nucleous comprising a water-immiscible medium, said polymeric layer comprising a discrete, gelled coacervate containing a low isoelectric point gelatin comprising a net negative charge and a derivative which comprises the reaction product of gelatin and a carboxylated gelatin derivatizing agent which will not substantially cross-link said gelatin, and which reacts with at least a portion of the amino groups of gelatin to provide neutralization of at least a portion of the positive charges provided to the gelatin molecule, in aqueous solution, by said amino groups, resulting in a derivatized gelatin material comprising a net negative charge.

4. A product as defined in claim 3 wherein said gelatin derivatizing agent comprises a dicarboxylic acid anhydride.

References Cited

UNITED STATES PATENTS

3,341,466 9/1967 Brynko et al. ----- 252—316

10 RICHARD D. LOVERING, Primary Examiner

U.S. Cl. X.R.

117—36.7, 62.2, 100 A; 264—4